

Patented Aug. 4, 1942

2,291,943

# UNITED STATES PATENT OFFICE

2,291,943

## PROCESS FOR PRODUCING HIGH SPEED CUTTING TOOLS

Lewis S. Bergen, Chappaqua, and Janet Z. Briggs, New York, N. Y., assignors to Crucible Steel Company of America, New York, N. Y., a corporation of New Jersey

No Drawing. Application April 23, 1941,  
Serial No. 389,884

### 1 Claim. (CL 148—21)

This invention pertains to improvements in relatively low alloy, tungsten- and molybdenum-containing, high speed cutting tools, characterized by high resistance to decarburization when subjected to hardening and tempering treatments in the absence of a protective coating, such as borax, etc., or a protective furnace atmosphere, such as nitrogen, etc., and to methods of so hardening and tempering such tools as to inhibit or prevent decarburization.

This application is a continuation in part of application Serial No. 301,776, filed October 28, 1939.

An object of the invention is to provide a cutting tool characterized as aforesaid and having cutting and other desirable properties of a high speed cutting tool which are commensurate of those of the high alloy, high tungsten types containing little or no molybdenum.

Based on long experience, cutting tools of the latter type, such as those made of the so-called "18-4-1" and "18-4-2" steels, etc., containing about 18% tungsten, about 4% chromium and 1 to 2% or so of vanadium, have assumed a commanding position in the high speed field due to combining such desirable qualities in service as high cutting performance, toughness, long life, etc., with such other desirable qualities in fabrication, as relative ease of heat treatment, resistance to decarburization, etc. Such tools have, however, the disadvantage of being relatively expensive because of their high content of alloys, particularly of tungsten, which is not only rather costly, but sometimes, as in case of war, difficult or impossible to secure in commercial quantities.

Accordingly, numerous proposals have been made to substitute the most closely related element, namely molybdenum, in whole or in part for tungsten in high speed steels, for cutting tools, and more recently in conjunction therewith to reduce the total alloy content. But tools of such steels have universally proved defective in comparison with the molybdenum-free, high tungsten types either as regards performance in service or as regards difficulties in fabrication or both, in consequence of which the high tungsten types have maintained their position despite their higher cost.

Of the many molybdenum containing, high speed analyses heretofore proposed for cutting tools, all of those which show performance ratings comparable to the high tungsten types, and hence are on a competitive basis therewith as regards this factor, are subject to serious surface decarburization, in the absence of special and expensive precautions, during the requisite heat treatments incident to conversion of the steel into finished tools ready for use. This decarburization, which results from exposure to the atmosphere when usual heat treating procedures are employed, may be overcome by excluding the atmosphere from contact with the metal while at elevated temperatures, as for example by a coating of borax or by heat treating in a salt bath or in a controlled atmosphere furnace, etc. But the added expense and delay of such procedures more than offset the advantage in lower first cost which such steels possess over the high tungsten types. Decarburization, on the other hand, is productive of a soft outer skin on the metal which must be cut or ground away at great expense before an acceptable cutting tool is obtained. Moreover, in some instances, this cannot be done owing to the complicated shape of the finished tool.

Now we have discovered, in accordance with a fundamental concept of our invention, that tools made of molybdenum containing high speed steels can be made inherently stable and completely resistant to decarburization during normal heat treatment, provided the aggregate content of tungsten and vanadium present in the steel is maintained sufficiently high in relation to the aggregate content of chromium and molybdenum. And we have further determined that if this relationship is maintained for steel containing chromium, tungsten, molybdenum and vanadium within the limits hereinafter specified, that not only is the resulting product as easy to fabricate into tools as are the high tungsten standards, such as 18-4-1, etc., but that the performance of such tools in service is in general equally good or better.

More specifically, we have determined that substantially complete resistance to decarburization is imparted to the tools during normal heat treating practices, if the ratio of tungsten

and vanadium to that of chromium and molybdenum is in excess of 0.77; that reasonably good stability is obtained if this ratio lies within the range of about 0.55 to 0.77; and that the steel becomes increasingly susceptible to decarburization as the ratio is progressively decreased below 0.55. This information may be summarized as follows, designating the ratio in question as the "stability ratio" or more briefly "S. R.":

$$S. R. = \frac{\%W + \%V}{\%Cr + \%Mo}$$

(a) over 0.77: steel completely stable  
(b) = 0.55 to 0.77: steel fairly stable  
(c) under 0.55: steel unstable

In the above formulation, the percentages of W, V, Cr and Mo refer to the percentages by weight of the total composition of the steel in which these constituents are present.

The relationships above summarized, which are based on actual tests, appear to rest on sound theoretical considerations. Tungsten-free molybdenum high speed steels are notoriously susceptible to decarburization when heat treated. This is due to the fact that the molybdenum and chromium carbides present are attacked by oxygen at relatively low temperatures, whereas the tungsten and vanadium carbides are stable at much higher temperatures. Based on these considerations, it may be inferred that molybdenum and chromium containing high speed steels may be stabilized by additions of tungsten and vanadium, sufficient to stabilize the carbides and prevent their attack by the atmosphere during heat treatment. Since other considerations than decarburization place rather definite restrictions on the vanadium content, the balance required to stabilize the steel may be effected by additions of tungsten.

As our tests have shown, it is not necessary that all of the carbon in the steel be present as tungsten and vanadium carbides, but only that a certain proportion be present in this form. Based on the test results presented below in Table II, it is found that if over 62% of the total carbon in the steel is present as carbides of tungsten and vanadium, that the steel will be stable; and that if this percentage lies between about 50 and 62%, the steel will not be completely resistant to decarburization under all conditions, but will be in most cases. On the other hand, steel for which the percentage is below about 50%, will be subject to decarburization in all heat treatments unless the surface is protected against atmospheric attack.

By normal heat treatment for tools in accordance with our invention, is meant hardening and tempering treatments in which the tools are first heated above the critical and at about 2100 to 2350° F., preferably at about 2175 to 2275° F., for an interval sufficient to austenitize and to produce sufficient carbide solution to give cutting performances comparable to those of the high tungsten steels, such as 18-4-1. Ordinarily, a relatively short time of heating at the aforesaid temperatures will suffice, i. e. a matter of minutes, for example about one to five minutes in the usual case, although heating at such temperatures for periods as high as one or two hours is permissible in some instances, following which the steel is rapidly cooled or quenched to harden, for example by air cooling or quenching in oil, or in a hot salt or lead bath, etc. The subsequent tempering is usually carried out by re-

heating up to about 950° to 1150° F. for about one to three hours.

The performance of the tools in service, i. e. their cutting ability, etc., follows closely the ratios above stated as applied particularly to analyses within the following limits:

|            | Per cent          |
|------------|-------------------|
| Carbon     | About 0.7 to 1.25 |
| Chromium   | About 3 to 8      |
| Molybdenum | About 2.5 to 7    |
| Tungsten   | About 3 to 10     |
| Vanadium   | About 1 to 6      |

15 We find that within these ranges, tools made of steels for which the stability ratio is above 0.77 show up in lathe tool tests from approximately equal to as much as 40% better than the 18-4-1 steel, depending on the analysis; that tools made of the steels for which this ratio is within the range of 0.55 to 0.77 are in general somewhat below the 18-4-1 in this respect; and that the lathe tool rating is considerably lower for steels having a stability ratio below 0.55, as evidenced by the data presented below in Table II for steels of the analyses given in Table I. Within the above limits, particularly good steels are found within the following preferred limits for the alloying constituents:

|            | Per cent         |
|------------|------------------|
| Carbon     | About 0.8 to 1.0 |
| Chromium   | About 3.0 to 4.5 |
| Molybdenum | About 2.5 to 6.0 |
| Tungsten   | About 3.5 to 7.0 |
| Vanadium   | About 1.0 to 3.0 |

Table I

| Steel | Analysis |     |     |     |     |      |
|-------|----------|-----|-----|-----|-----|------|
|       | C        | Cr  | Mo  | W   | V   | Bal. |
| 45 1  | 1.13     | 4.2 | 3.7 | 7.6 | 2.5 | Fe   |
| 2     | 0.91     | 4.1 | 3.4 | 7.5 | 1.4 | Fe   |
| 3     | 0.92     | 4.1 | 3.5 | 6.8 | 2.0 | Fe   |
| 4     | 0.95     | 4.4 | 4.1 | 7.3 | 2.2 | Fe   |
| 5     | 1.03     | 4.0 | 3.6 | 5.5 | 2.6 | Fe   |
| 6     | 1.20     | 3.6 | 3.6 | 3.6 | 3.8 | Fe   |
| 7     | 1.32     | 4.1 | 3.4 | 4.2 | 3.7 | Fe   |
| 8     | 0.90     | 4.2 | 3.7 | 6.7 | 1.3 | Fe   |
| 9     | 1.09     | 4.0 | 3.5 | 4.4 | 3.0 | Fe   |
| 10    | 0.96     | 4.2 | 3.8 | 5.6 | 1.9 | Fe   |
| 11    | 0.91     | 4.3 | 3.6 | 5.7 | 1.5 | Fe   |
| 12    | 1.12     | 4.1 | 3.8 | 3.7 | 3.4 | Fe   |
| 13    | 0.86     | 4.2 | 6.3 | 8.1 | 1.3 | Fe   |
| 14    | 1.30     | 4.1 | 3.6 | 3.6 | 3.3 | Fe   |
| 15    | 1.11     | 4.2 | 3.8 | 3.5 | 3.4 | Fe   |
| 16    | 1.12     | 4.0 | 3.5 | 3.5 | 2.8 | Fe   |
| 17    | 1.09     | 4.1 | 3.5 | 3.6 | 2.8 | Fe   |
| 18    | 0.97     | 4.1 | 3.5 | 3.5 | 2.7 | Fe   |
| 19    | 0.96     | 4.3 | 3.6 | 4.4 | 2.0 | Fe   |
| 20    | 1.04     | 4.1 | 3.9 | 4.3 | 2.3 | Fe   |
| 21    | 0.96     | 4.2 | 3.5 | 3.5 | 2.5 | Fe   |
| 22    | 0.87     | 4.2 | 3.8 | 4.8 | 1.3 | Fe   |
| 23    | 0.88     | 4.1 | 3.6 | 3.5 | 2.4 | Fe   |
| 24    | 1.02     | 4.1 | 3.5 | 3.4 | 2.4 | Fe   |
| 25    | 1.06     | 4.2 | 3.0 | 2.5 | 2.8 | Fe   |
| 26    | 0.95     | 4.0 | 3.6 | 3.7 | 1.7 | Fe   |
| 27    | 0.85     | 4.0 | 3.6 | 3.6 | 1.7 | Fe   |
| 28    | 0.78     | 4.1 | 3.6 | 3.6 | 1.7 | Fe   |
| 29    | 0.88     | 4.2 | 6.4 | 5.5 | 1.5 | Fe   |
| 30    | 0.87     | 4.2 | 3.6 | 3.5 | 1.5 | Fe   |
| 31    | 0.95     | 4.1 | 3.7 | 2.9 | 2.1 | Fe   |
| 32    | 1.01     | 4.4 | 3.8 | 2.7 | 2.0 | Fe   |
| 33    | 0.91     | 4.3 | 6.7 | 4.6 | 1.5 | Fe   |
| 34    | 0.87     | 4.2 | 3.7 | 2.8 | 1.5 | Fe   |
| 35    | 1.03     | 4.2 | 4.0 | 1.4 | 2.8 | Fe   |
| 36    | 0.89     | 4.2 | 6.5 | 3.5 | 1.4 | Fe   |
| 37    | 0.93     | 4.1 | 4.0 | 1.4 | 2.1 | Fe   |
| 38    | 0.91     | 4.3 | 6.3 | 2.4 | 1.5 | Fe   |
| 39    | 0.85     | 4.2 | 3.5 | 1.8 | 1.4 | Fe   |
| 40    | 1.08     | 4.2 | 3.8 | 0.0 | 2.8 | Fe   |
| 41    | 0.90     | 4.1 | 3.6 | 0.0 | 2.1 | Fe   |
| 42    | 0.86     | 4.2 | 6.5 | 1.5 | 1.5 | Fe   |
| 43    | 0.84     | 4.2 | 3.7 | 0.0 | 1.5 | Fe   |
| 44    | 0.83     | 4.0 | 6.2 | 0.0 | 1.5 | Fe   |

Table II

| Steel | Stability ratio<br>% W + % V<br>% Cr + % Mo | Decarburization<br>after the above-<br>mentioned<br>normal heat<br>treatment |              | Lathe tool<br>rating vs.<br>18-4-1-<br>18-4-1=100 |
|-------|---------------------------------------------|------------------------------------------------------------------------------|--------------|---------------------------------------------------|
|       |                                             | Measured<br>depth of—                                                        | File<br>test |                                                   |
| 1.    | 1.28                                        | None                                                                         | A            |                                                   |
| 2.    | 1.17                                        | None                                                                         | A            |                                                   |
| 3.    | 1.13                                        | None                                                                         | A            |                                                   |
| 4.    | 1.12                                        | None                                                                         | A            |                                                   |
| 5.    | 1.06                                        | None                                                                         | A            |                                                   |
| 6.    | 1.05                                        | None                                                                         | A            | 134                                               |
| 7.    | 1.05                                        | None                                                                         | A            | 93                                                |
| 8.    | 1.00                                        | None                                                                         | A            | 99                                                |
| 9.    | 0.99                                        | None                                                                         | A            | 110                                               |
| 10.   | 0.94                                        | None                                                                         | A            | 116                                               |
| 11.   | 0.91                                        | None                                                                         | A            | 100                                               |
| 12.   | 0.91                                        | None                                                                         | A            | 100                                               |
| 13.   | 0.89                                        | None                                                                         | A            |                                                   |
| 14.   | 0.88                                        | None                                                                         | A            | 91                                                |
| 15.   | 0.85                                        | None                                                                         | A            | 139                                               |
| 16.   | 0.84                                        | None                                                                         | A            | 133                                               |
| 17.   | 0.83                                        | None                                                                         | B            | 139                                               |
| 18.   | 0.82                                        | None                                                                         | A            | 111                                               |
| 19.   | 0.82                                        | None                                                                         | B            |                                                   |
| 20.   | 0.82                                        | None                                                                         | A            |                                                   |
| 21.   | 0.78                                        | None                                                                         | B            | 116                                               |
| 22.   | 0.77                                        | None                                                                         | B            |                                                   |
| 23.   | 0.76                                        | None                                                                         | C            | 105                                               |
| 24.   | 0.76                                        | None                                                                         | A            | 126                                               |
| 25.   | 0.72                                        | None                                                                         | B            |                                                   |
| 26.   | 0.71                                        | None                                                                         | A            | 73                                                |
| 27.   | 0.70                                        | None                                                                         | A            | 78                                                |
| 28.   | 0.70                                        | None                                                                         | B            | 82                                                |
| 29.   | 0.65                                        | None                                                                         | B            |                                                   |
| 30.   | 0.65                                        | None                                                                         | C            | 78                                                |
| 31.   | 0.64                                        | None                                                                         | B            | 120                                               |
| 32.   | 0.57                                        | None                                                                         | B            |                                                   |
| 33.   | 0.55                                        | None                                                                         | B            |                                                   |
| 34.   | 0.52                                        | 0.0014                                                                       | C            |                                                   |
| 35.   | 0.51                                        | 0.0004                                                                       | C            |                                                   |
| 36.   | 0.46                                        | 0.0020                                                                       | B            |                                                   |
| 37.   | 0.43                                        | 0.0009                                                                       | D            |                                                   |
| 38.   | 0.37                                        | 0.0012                                                                       | C            |                                                   |
| 39.   | 0.36                                        | 0.0007                                                                       | C            |                                                   |
| 40.   | 0.35                                        | 0.0018                                                                       |              | 72                                                |
| 41.   | 0.27                                        | 0.0020                                                                       | D            | 70                                                |
| 42.   | 0.27                                        | 0.0009                                                                       | D            |                                                   |
| 43.   | 0.19                                        | 0.0014                                                                       | D            |                                                   |
| 44.   | 0.14                                        | 0.0048                                                                       | D            |                                                   |

In the lathe tool ratings of the above Table II, the value of the tool is measured by the elapsed time of cutting before failure under conditions where speed, depth of cut and rate of feed are maintained constant. For comparative purposes, cutting tests were made on a heat treated chromium-nickel steel log having a Brinell hardness of 220-240, employing cutting tools made of each of the steels for which lathe

tool ratings are given in Table II, and also with tools made of the 18-4-1 steel. The ratings given in the last column of Table II are expressed on a comparative basis in terms of a rating of 100 for the 18-4-1 steel. The file test ratings given in Table II were of the usual type, in which the rating A represents steels on which the file made no impress when drawn across them; rating B is accorded to steels on which the file had an extremely slight drag; rating C those for which the file had a definite bite into the steel; and rating D, steels for which the file had a pronounced bite representing a soft outer skin.

In general, the balance of the alloy, aside from those above specified in the proportions stated, will consist substantially of iron except for the usual tolerances for impurities and such elements unavoidably present in small amounts, as manganese, silicon, etc. Silicon in excess of about 0.5% is found to be detrimental to the cutting properties of the steel, and hence is preferably held under this figure.

The alloy is preferably made by melting the constituents in the usual manner in the electric or crucible furnace, casting into ingots, and hot working the ingots by forging, rolling, etc. The steel is then made into cutting tools in the usual way, and the tools heat treated in the manner above described.

30 We claim:

A process for minimizing surface decarburization of molybdenum high speed steel during heating for hot working, hardening and the like, which comprises: forming the steel of an alloy containing about 0.7 to under 1.25% carbon, about 3 to 8% chromium, about 2.5 to 7% molybdenum, about 3 to 10% tungsten, about 1 to 6% vanadium, under 0.5% silicon, and the balance substantially all iron, in which the ratio of tungsten plus vanadium to molybdenum plus chromium exceeds 0.77, and subjecting the steel to elevated temperature for hot working, hardening and related treatments, in the absence of special precautions including the use of protective fluxes, controlled furnace atmospheres and the like, for protecting the steel against surface decarburization.

LEWIS S. BERGEN.  
JANET Z. BRIGGS.